

March 17, 1964

J. G. MURRAY ET AL  
COMPOSITIONS OF MATTER AND USES OF SAID  
COMPOSITIONS IN A PROJECTION SYSTEM  
Filed June 5, 1962

3,125,634



Fig. 2.

Inventors:  
 James G. Murray;  
 Frederick F. Holub,  
 Matthew J. Smith,  
 by Joseph T. Colon  
 Their Attorney.

3,125,634  
**COMPOSITIONS OF MATTER AND USES OF SAID COMPOSITIONS IN A PROJECTION SYSTEM**  
 James G. Murray and Frederick F. Holub, Scotia, and Matthew J. Smith, Schenectady, N.Y., assignors to General Electric Company, a corporation of New York  
 Filed June 5, 1962, Ser. No. 200,074  
 11 Claims. (Cl. 173—7.3)

This invention is concerned with compositions of matter and their use in projection systems utilizing these compositions of matter as deformable media. More particularly, the invention is concerned with compositions of matter having the general formula

I



where R is a monovalent hydrocarbon radical selected from the class consisting of the methyl and phenyl radicals, Z is a radical selected from the class consisting of the biphenyl, naphthyl, and phenoxyphenyl radicals, and n is an integer equal to from 2 to 4, inclusive. The invention also relates to the use of the aforesaid compositions of matter as the deformable medium in a projection system which is more particularly disclosed in U.S. 2,943,147, issued June 28, 1960, and in U.S. 2,391,450, issued December 25, 1945.

In the aforesaid U.S. Patent 2,943,147, assigned to the same assignee as the present invention, there is disclosed and claimed a projection system employing a deformable medium having a high resistivity which is responsive to an electron beam which is velocity modulated. In general, this apparatus which is illustrated in FIGURE 1 of the attached drawing comprises an evacuated glass envelope 10 containing an electron gun 11 for producing an electron beam 13 and deflecting it in a rectangular raster over the surface of a transparent, deformable medium 15 that is within a portion 17 of the transparent container; an enlarged view of this portion of the assembly is shown in FIGURE 2. The beam 13 is preferably velocity modulated by a television signal that is applied to the deflection means (not shown) in the electron gun 11. The deformable medium 15 has a center portion 19 of decreased thickness, coincident with the raster area of the beam 13, which is produced by electrons from the beam 13 that are attracted to a conducting coating 21 on the inner surface of the container 17. These electrons also produce deformations in the surface of the deformable medium 15, the amplitudes of which are a function of the number of electrons deposited by the beam 13 at the various points on the surface of the medium 15. Consequently, the amplitudes of these deformations are a function of the television signal modulating electron beam 13.

These deformations are utilized to diffract light from a light source 23 in an optical system which is illustrated as including a lens 24 that images light source 23 on the surface of medium 15 through a bar and slit system 25. Another lens 29 images the slits of system 25 on the bars of another bar and a slit system 31 in the absence of deformations in the surface of the deformable medium. However, any deformations phase diffract the light so that it passes through the slits in the system 31 with an intensity that corresponds to the amplitudes of the deformations and thus the amplitude of the applied television signal. The light passing through system 29 is imaged by a projection lens 33 on a screen 35 after reflection from a mirror 37.

If a conventional deformable medium is utilized in the illustrated system, the average charge density produces a force on the medium 15 that overcomes the surface tension from the excess medium outside the raster area and decreases the portion 19 of medium 15 to zero thickness; under such conditions, no deformations can be formed and the system becomes inoperative until the medium is replaced.

In this U.S. Patent 2,943,147, it is stated that if the medium has the property of decreasing in resistivity with decreasing thickness, portion 19 does not decrease to zero thickness under the pressure of the charges but rather maintains a thickness the value of which is a function of the magnitude of charge density on the surface of the medium 15. With a decrease in resistivity, the time constant is decreased for the passage of leakage current from the surface of the deformable medium 15 to the conducting coating 21 beneath it, resulting in increase in leakage current, which decreases the charge density on the surface of the medium, thereby relieving the pressure somewhat. Ultimately, an equilibrium condition is attained in which the pressure from the charges on the surface of the medium equals the pressure from the surface tension on the excess medium around the raster. Then the thickness at this equilibrium condition is maintained. The charge density on the surface of the medium never decreases to zero due to the leakage because it is continually being replaced by the electrons from the beam 13.

The deformable compositions described in the aforesaid Patent U.S. 2,943,147 as suitable for the medium are required to be transparent, be capable of withstanding electron bombardment without significant decomposition, have a viscosity at the operating temperature (between about 25° C. and 150° C.) of approximately 100 to 50,000 centistokes, and the deformable composition must not decompose the conducting coating. The medium must also have a resistivity that varies within the range of approximately  $10^{14}$  to  $10^{11}$  ohms-cm., with the average resistivity at the stable thickness being approximately  $10^{11}$  ohms-cm.

Among the deformable media or fluids described in this patent are, for instance, beeswax, methyl silicone fluids, methylsilicone fluids containing up to 5% of phenyl silicones, methylphenyl silicones containing an average of two methyl and phenyl groups per silicon atom in which the mol ratio of methyl groups to silicon atoms is greater than 0 and less than 2, etc. However, it has been found that these deformable fluids are not as stable as one would desire because under the influence of an electron beam, the deformable fluid tends to increase in viscosity, and with continued use in the projection system described above, the viscosity increases to a point where gel particles begin to form and ultimately the deformable medium gels; of course, this means that the apparatus can no longer be used with that particular deformable medium.

Unexpectedly, we have discovered that a group of organic compositions of Formula I described previously, is eminently suitable as the deformable medium in the above-described projection system. Not only are sharp, viewable images of good light intensity obtained with these fluids, but also these fluids have exceptionally low vapor pressure and much greater resistance to irradiation, and therefore are more stable in the presence of the electron beam used in the aforesaid projection system. The compositions employed by us in the aforesaid projection system can be used continuously for much longer periods of time without significant change in the deformable medium, thus adding greatly to the life of the projection system.

Within the scope of Formula I described above, the following examples are given by way of illustration and not by way of limitation as to the preparation of a large number of these compositions which can be employed as the deformable medium in the aforesaid projection system. It is to be understood that where the biphenylyl or phenoxyphenyl radical is present in the composition used as the deformable medium, the phenyl radicals of the biphenylyl group and the phenoxy radical of the phenoxyphenyl group may be ortho-, meta- or para- to the point of attachment in the biphenylyl or in the phenoxyphenyl radical shown in Formula I. Thus, the biphenylyl radical attachments may be illustrated as



and the phenoxyphenyl radical attachments may be illustrated as



The naphthyl radical can be attached in either the  $\alpha$  or  $\beta$  positions.

#### EXAMPLE 1

The composition 1,3-di(o-phenylphenoxy)-1,3-diphenyl-1,3-dimethylsiloxydisiloxane having the formula

II



was prepared as follows. o-Phenylphenoxyphenylmethylchlorosilane was first prepared by adding a solution of 85.1 grams of o-phenylphenol in benzene (180 ml. of solution) to a stirred mixture of 95.6 grams of phenylmethyldichlorosilane in 250 ml. benzene and 39.6 grams of dry pyridine at 0 to 10° C. over a period of 40 minutes. The mixture was stirred for an additional 2 hours and thereafter filtered. The filter cake was washed with benzene and the benzene wash was added to the filtrate and benzene was removed by distillation. The residue was then distilled under reduced pressure to yield 113 grams of a product boiling at 149-156° C./0.1 mm., which was identified as o-phenylphenoxyphenylmethylchlorosilane. About 65 grams of this latter chlorosilane was dissolved in 100 ml. of benzene and to this was added 1.8 grams of water (sufficient to hydrolyze completely the silicon-bonded chlorine) in 15.8 ml. pyridine over a period of 2 hours at a temperature of 20-30° C. The mixture was stirred for 18 hours, filtered and the filter cake washed with benzene. The benzene wash and the filtrate were combined and fractionally distilled to remove benzene and to yield a residue which distilled at 250-260° C./0.1 mm. This composition was identified as having the formula II by the fact that it was found to contain 77.0% carbon, 5.9% hydrogen and 9.7% silicon, as contrasted to the theoretical values of 76.72% carbon, 5.76% hydrogen and 9.44% silicon.

#### EXAMPLE 2

This example illustrates the preparation of compound bis - (o-phenylphenoxyphenylmethylsiloxy)diphenylsilane having the formula

III



More particularly, 11.1 grams of diphenylsilanediol was added in small portions over a period of 20 minutes to a mixture of 33.7 grams of o-phenylphenoxyphenylmethylchlorosilane (prepared in accordance with the directions in Example 1) dissolved in 100 ml. benzene and 10 ml. pyridine. The temperature during this addition was kept at around 20-30° C. After allowing the resulting mixture to stand with stirring for about 18 hours, the product was filtered, the benzene removed from the filtrate by distillation, and the residue then fractionally distilled under reduced pressure to yield a product having a boiling point of 273-276° C./0.05 mm. This material was found to be the composition identified by Formula III as evidenced by the fact that it contained 75.9% carbon, 5.9% hydrogen, and 10.2% silicon as contrasted to the theoretical values of 75.71% carbon, 5.59% hydrogen, and 10.62% silicon.

#### EXAMPLE 3

1,5-di(o-phenylphenoxy)-1,5-diphenyl-1,3,5-tetramethyltrisiloxane having the formula

IV



was prepared as follows. The intermediate chlorosilane required, namely o-biphenylyloxyphenylmethylchlorosilane, was prepared in accordance with the method described in Example 1. This o-biphenylyloxyphenylmethylchlorosilane was then hydrolyzed by adding 130 grams of this material to a mixture of 100 grams of sodium bicarbonate in 400 ml. acetone held at a temperature -15 to -20° C. Addition was completed in 15 minutes and stirring of the mixture was continued for an additional hour at the same temperature. The resulting mixture was filtered and acetone removed under reduced pressure at room temperature. The resulting mixture was then subjected to a reduced pressure of 0.5 mm. at room temperature. This hydrolyzate (which was the o-biphenylyloxyphenylsilanol) was added over a period of 45 minutes to a solution of 25.8 grams dimethyldichlorosilane and 31.6 grams pyridine and 200 ml. benzene at 0-10° C. The mixture was stirred for approximately 3 hours and thereafter allowed to warm up to room temperature. The benzene was removed and the product fractionally distilled under reduced pressure to yield a liquid boiling at 251-274° C./0.08 mm.,  $n_D^{20}=1.5876$ . This composition was then stirred with a solid sodium bicarbonate to remove small amounts of unreacted chlorosilanes and thereafter the sodium bicarbonate was removed and the product fractionally distilled to yield a composition boiling at 248-266° C./0.06 mm.,  $n_D^{20}=1.5901$ . This material which had a viscosity at 25° C. of 900 centistokes was identified as the above-identified

composition having Formula IV as evidenced by the fact that it was found to contain 73.5% carbon, 6.3% hydrogen, 11.4% silicon and to have a molecular weight of 613 as contrasted to the theoretical values of 71.8% carbon, 6.0% hydrogen, 12.6% silicon and a molecular weight of 669.

#### EXAMPLE 4

The composition 1,3-di(m-phenoxyphenoxy)-1,3-di-phenyl-1,3-dimethylsiloxane having the formula

V



was prepared as follows. The chlorosiloxane intermediate, namely, chloromethylphenyldisiloxane having the formula

VI



was prepared by adding 18 grams of water over a 3 hour period to a stirred solution of 709 grams methylphenyl-dichlorosilane in an equal weight of diethyl ether at 10° C. Ether was evaporated and the product was fractionally distilled under reduced pressure to yield the above chlorosiloxane product boiling at 120-121.5° C./0.02 mm. About 65.4 grams of the aforesaid chloromethyl-phenyldisiloxane was added dropwise over a 2 hour period to a reaction vessel containing 33.4 grams m-phenoxy-phenol and 34.8 grams pyridine in 200 ml. benzene as solvent. After heating the mixture of ingredients at the reflux temperature of the mass for 2 hours, the pyridine hydrochloride was filtered off and washed with benzene. The solvent was removed from the filtrate and distillation under reduced pressure yielded 102.0 grams of a liquid of the above Formula V, boiling at 265-268° C./0.01 mm.,  $n_{D}^{20}=1.5943$ . Analysis of this composition showed it to contain 72.3% carbon, 5.6% hydrogen and to have a molecular weight of 618, as contrasted to the theoretical values of 72.79% carbon, 5.47% hydrogen and a molecular weight of 627.

#### EXAMPLE 5

The composition 1,3-di( $\beta$ -naphthoxy)-1,1,3,3-tetraphenyl disiloxane having the formula

VII



is prepared similarly as above by first reacting 1 mole of  $\beta$ -naphthol with 1 mole diphenyldichlorosilane in pyridine as a hydrohalide acceptor at a temperature of about 0° C. to give  $\beta$ -naphthoxy diphenylchlorosilane. This chlorosilane was then hydrolyzed in the usual fashion with water to give the above-identified composition having Formula VII.

#### EXAMPLE 6

The composition 1,5-di( $\alpha$ -naphthoxy)-1,5-diphenyl-1,3,5-tetramethyltrisiloxane having the formula

VIII



is prepared in the same manner as described in Examples 1 and 2. More particularly, the  $\alpha$ -naphthoxy phenylmethylchlorosilane required for preparation of the composition of Formula VIII is prepared by the same procedure as used in Example 1 to prepare  $\alpha$ -phenylphenoxy-phenylmethylchlorosilane, but instead of using  $\alpha$ -phenyl-phenol,  $\alpha$ -naphthol is used. The obtained  $\alpha$ -naphthoxy-phenylmethylchlorosilane is hydrolyzed similarly as in Example 3 to give the  $\alpha$ -naphthoxy-methylphenylsilanol. The latter silanol was then added similarly again as in Example 3, to dimethylchlorosilane employing the same molar concentrations and the same conditions, to yield the desired composition having Formula VIII.

In order to determine (by means of an accelerated test) the radiation resistance of the aforesaid compositions in an electron beam which would be the conditions under which these fluids would be expected to operate in the above-described projection system, the fluids prepared in the above examples were subjected to electron irradiation with a 1500 kv. resonant transformer at a current input of 200-500 microampères at a dose of  $20-50 \times 10^6$  roentgens/minute to a total dose of 400 megaroentgens. The following Table I shows the total number of molecules of gas per 100 electron volts absorbed (identified as "G gas"), as well as the change in viscosity (in centistokes) prior to irradiation (identified as " $\eta_0$ , cs.") and after irradiation (identified as " $\eta$ , cs.") at the temperature at which irradiation was measured.

Table I

| Composition of Example | G gas | $\eta_0$ , cs. |       | $\eta$ , cs. |       |
|------------------------|-------|----------------|-------|--------------|-------|
|                        |       | Temp., °C.     | Visc. | Temp., °C.   | Visc. |
| 35                     |       |                |       |              |       |
| 1                      | 0.03  | 50             | 230   | 50           | 313   |
| 2                      | 0.026 | 50             | 530   | 50           | 747   |
| 3                      | 0.057 | 25             | 900   | 25           | 1350  |
| 40                     | 0.05  | 25             | 400   | 25           | 628   |

The low gas value and the small change in viscosity under the accelerated test conditions applied to the above-identified compositions as shown in Table I above establish the eminent suitability of these compositions as the deformable medium in place of deformable media disclosed in the aforesaid U.S. Patent 2,943,147. To further establish the usefulness of the compositions of the above type, the composition of Example 4 was subjected to an electron-raster test using 10 kv. and 2 to 3 microampères. This test involved subjecting the deformable fluid to constant electron irradiation for a time until first evidence of gelation (called "incipient gel formation") was noted. This is an accelerated, severe test because in the normal use of the aforesaid apparatus, the deformable medium would be constantly replenished and removed from the zone of irradiation. It was found that the aforesaid composition when subjected to this severe test did not show any incipient gel formation until after 135 minutes, indicating its eminent stability under irradiation conditions.

As a still further test, the compositions of Examples 3 and 4 were used in the normal fashion in the apparatus described in the attached drawing and in U.S. 2,943,147 as the deformable medium recited in the drawing and patent. It was found that sharp, viewable images of good light and color intensity were obtained in each instance.

In addition to the uses described above, the polysiloxanes of Formula I can also be used as hydraulic and dielectric fluids where thermal stability and radiation resistance are prerequisites. In sealed systems, the eminent resistance to elevated temperatures recommends these materials as hydraulic fluids in automobiles and in airplanes.

In addition, because of the radiation resistance of the aforesaid compositions, they are especially useful in outer space application.

When employing the aforesaid compositions of Formula I as the deformable medium in the above-identified projection system, it will be apparent to those skilled in the art that in addition to using the compositions described above alone, they may be mixed with other suitable compositions used as the deformable medium. Thus, these compositions can be mixed with other organopolysiloxanes (such as those disclosed in Rochow Patents U.S. 2,258,221 and 2,258,222) in varying amounts and can be used to modify the organopolysiloxanes disclosed in the aforesaid U.S. Patent 2,943,147.

The compositions of the present invention may be prepared by methods well known in the art. Generally, in making the disiloxanes, reaction is advantageously carried out by hydrolyzing a composition having the formula



where Z and R have the meanings given above, and X is a hydrolyzable group, for instance, halogen, such as chlorine, bromine, etc. Generally, this hydrolysis is effected, usually in the presence of a hydrohalide acceptor, by adding a sufficient amount of water to the composition of Formula IX to effect complete hydrolysis of the silicon-bonded hydrolyzable group.

When making polysiloxane compositions of the present invention having more than two siloxy units in the molecule (such as illustrated in Examples 2 and 3), reaction is advantageously carried out between 2 moles of the composition of Formula IX with 1 mole of a polysiloxane-diol of formula



where R has the meaning given above and m is a whole number equal to from 1 to 2. Alternatively, such composition can be obtained by reacting a compound of the formula



with a diorganosilane of the formula  $\text{R}_2\text{SiCl}_2$  where Z and R have the meanings given above.

The intermediate compositions having the formula



can be obtained by reacting 1 mole of a hydroxyaromatic compound of the formula  $\text{ZOH}$  with 1 mole of a diorganodichlorosilane (or mixture of diorganodichlorosilanes) of the formula  $\text{R}_2\text{SiCl}_2$  where Z and R have the meaning given above. In those instances where a chlorosilane is being reacted with a silanol or a polysiloxane-diol, it is advantageous also to employ a hydrohalide acceptor such as pyridine, tertiary amines, etc. The usual methods of fractional distillation and crystallization are employed to isolate the desired products.

In addition to the compositions described above in the preceding examples, other compositions may also be employed using the methods of preparation described both generically and specifically in the aforesaid examples. Among such other compositions which may be obtained in accordance with the practice of the present invention

may be mentioned compounds having the following formulas:

XII



XIII



XIV



What we claim as new and desire to secure by Letters Patent of the United States is:

1. A composition of matter having the general formula



where R is a member selected from the class consisting of methyl and phenyl radicals, Z is a member selected from the class consisting of biphenyl, naphthyl and phenoxyphenyl radicals and n is a whole number equal to from 2 to 4, inclusive.

2. A composition of matter having the formula



3. A composition of matter having the formula



4. A composition of matter having the formula



5. A composition of matter having the formula



6. A composition of matter having the formula



7. A projection system comprising a container having a conducting interior, a deformable medium in said container comprising a composition having the formula



where R is a member selected from the class consisting of the methyl radical and phenyl radical, Z is a member selected from the class consisting of the biphenyl, phenoxyphenyl, and naphthyl radicals, n is a whole number equal to from 2 to 4, inclusive, an electron beam means for producing an electrical charge on the surface of said deformable medium as a function of an applied electrical signal and cooperating with said conducting interior to subject the medium to a deforming force to produce deformations on the surface of said medium, and a light and optical system for projecting light as a function of the deformations in the surface of said medium.

8. A projection system comprising a container having a conducting interior, a deformable medium in said container comprising a composition having the formula



an electron beam means for producing an electrical charge on the surface of said deformable medium as a function of an applied electrical signal and cooperating with said conducting interior to subject the medium to a deforming force to produce deformations in the surface of said medium, and a light and optical system for projecting light as a function of the deformations in the surface of said medium.

9. A projection system comprising a container having a conducting interior, a deformable medium in said container comprising a composition having the formula



an electron beam means for producing an electrical charge on the surface of said deformable medium as a function of an applied electrical signal and cooperating with said conducting interior to subject the medium to a deforming force to produce deformations in the surface of said medium, and a light and optical system for projecting light as a function of the deformations in the surface of said medium.

10. A projection system comprising a container having a conducting interior, a deformable medium in said container comprising a composition having the formula



an electron beam means for producing an electrical charge on the surface of said deformable medium as a function of an applied electrical signal and cooperating with said conducting interior to subject the medium to a deforming force to produce deformations in the surface of said medium, and a light and optical system for projecting light as a function of the deformations in the surface of said medium.

11. A projection system comprising a container having a conducting interior, a deformable medium in said container comprising a composition having the formula



an electron beam means for producing an electrical charge on the surface of said deformable medium as a function of an applied electrical signal and cooperating with said conducting interior to subject the medium to a deforming force to produce deformations in the surface of said medium, and a light and optical system for projecting light as a function of the deformations in the surface of said medium.

No references cited.